

# United States Patent [19]

Hara et al.

[11] 3,861,923

[45] Jan. 21, 1975

[54] **SILVER HALIDE COLOR PHOTOGRAPHIC MATERIALS CONTAINING A 3-UREIDO-5-PYRAZOLONE COUPLER AND AN ALDEHYDE COMPOUND**

[75] Inventors: **Hiroshi Hara; Yukio Yokota; Hiroyuki Amano; Tokio Nishimura,** all of Kanagawa, Japan

[73] Assignee: **Fuji Photo Film Co., Ltd.,** Kanagawa, Japan

[22] Filed: **May 31, 1973**

[21] Appl. No.: **365,678**

## [30] Foreign Application Priority Data

May 31, 1972 Japan ..... 47-54500

[52] U.S. Cl. .... **96/100, 96/56, 96/74,**  
96/111

[51] Int. Cl. .... **G03c 1/40**

[58] Field of Search ..... 96/100, 56, 111

## [56] References Cited

### UNITED STATES PATENTS

2,518,686 8/1950 Harsh et al. .... 96/56

|           |        |                     |        |
|-----------|--------|---------------------|--------|
| 3,140,177 | 7/1964 | Welch.....          | 96/56  |
| 3,393,071 | 7/1968 | Monbaliu et al..... | 96/100 |
| 3,468,666 | 9/1969 | Shiba et al.....    | 96/100 |
| 3,558,319 | 1/1971 | Hamaoka et al.....  | 96/100 |

## OTHER PUBLICATIONS

Croome et al., Photographic Gelatin, page 18, Focal Press, N.Y., 1965.

Primary Examiner—J. Travis Brown  
Attorney, Agent, or Firm—Sughrue, Rothwell, Mion,  
Zinn & Macpeak

## [57] ABSTRACT

Color photographic materials forming magenta dye images of excellent heat and moisture resistance comprising a support having a silver halide photographic emulsion layer containing a 3-ureido-5-pyrazolone magenta coupler together with a compound having an aldehyde group bonded to a carbon atom.

**21 Claims, No Drawings**

**SILVER HALIDE COLOR PHOTOGRAPHIC  
MATERIALS CONTAINING A  
3-UREIDO-5-PYRAZOLONE COUPLER AND AN  
ALDEHYDE COMPOUND**

## BACKGROUND OF THE INVENTION

## 1. Field of the Invention

The present invention relates to color photography, more particularly, it relates to a color photographic material capable of forming magenta dye images of good heat and moisture resistance.

## 2. Description of the Prior Art

It is well known in the field of color photography that cyan, magenta and yellow color images are formed by the coupling of the oxidation product of an aromatic primary amino developing agent and color forming couplers. It is also known that various pyrazolone derivatives can be used for forming magenta color images.

The magenta dye images are ordinarily unstable to heat and moisture, and when they are exposed to heat or moisture or are stored for a long period of time, the low density portions of the magenta dye images tend to fade. It is known that such a phenomenon occurs due to unreacted coupler remaining in the color photographic material, and, thus, the aforesaid tendency is particularly seen at low density image portions where a large amount of unreacted coupler remains (see, e.g., P. W. Vittum; *Journal of the American Chemical Society*; Vol. 72, 1533(1950)).

Various methods for preventing fading of magenta dye images have been proposed. For instance, according to the method described in U.S. Pat. No. 3,140,177, a color photographic material is processed in an acid processing solution containing formalin as the final processing step of the color photographic material. However, such a method is undesirable since formalin gives off a bad odor and further it can be harmful to the body.

According to U.S. Pat. No. 3,468,666, a bispyrazolone prepared by the condensation of 3-acylamino-5-pyrazolone and an aldehyde is used as the magenta coupler. However, such a bispyrazolone has the fault that it does not give a sufficient coupling density upon color development. Furthermore, the dye image formed by such a bispyrazolone is not very fast to heat and moisture.

Accordingly, the development of new means for forming magenta dye images of good fastness to heat and moisture has been desired.

## SUMMARY OF THE INVENTION

One object of this invention is, therefore, to provide a color photographic material capable of forming fast magenta images.

It has been discovered that the above mentioned object of this invention can be attained by using a 3-ureido-5-pyrazolone and a compound having an aldehyde group bonded to a carbon atom. Thus, according to the present invention, a silver halide photographic emulsion containing a 3-ureido-5-pyrazolone type magenta coupler and a compound having an aldehyde group bonded to a carbon atom is presented.

## DETAILED DESCRIPTION OF THE INVENTION

According to one embodiment of this invention, there is provided a color photographic material com-

prising a support having coated thereon a silver halide emulsion layer containing at least one of the non-diffusible 3-ureido-5-pyrazolones represented by the following general formula I



wherein  $R_1$  represents an alkyl group or an aryl group and  $R_2$  represents a phenyl group and at least one of a compound having an aldehyde group bonded to a carbom atom

The term "non-diffusible" in this specification has its well known meaning as it is used for color couplers in the field of color photography, i.e., it means that the coupler does not substantially move in the colloid layers of a photographic material in the presence of an aqueous alkaline processing solution.

When  $R_1$  represents an alkyl group, most generally the alkyl group will have 1 to 32 carbon atoms, though this range is not limitative. It is most preferred that when  $R_1$  is an alkyl group it have 8 to 18 carbon atoms, since an alkyl group with 8 or more carbon atoms acts as a ballasting group, while alkyl groups of 19 or more carbon atoms are not preferred from an industrial stand point, i.e., the compounds have an increased production cost, difficulty of synthesis, etc.

When  $R_1$  is an aryl group, it is monoaryl as exemplified in the following paragraphs.

When  $R_2$  represents a substituted phenyl group, preferred substituents include halogen, cyano, nitro, alkyl of 1-18 carbon atoms, alkoxy of 1-18 carbon atoms, aryl, e.g., phenyl, tolyl, etc., aryloxy, e.g., phenoxy, etc., carbamoyl, sulphamoyl, sulphonamido or acyl.

Specific examples of  $R_2$  include phenyl, 2-chlorophenyl, 4-chlorophenyl, 2,5-dichlorophenyl, 2,6-dichlorophenyl, 2,4,6-trichlorophenyl, 2-bromophenyl, 3,5-dibromophenyl, 2-cyanophenyl, 3-nitrophenyl, 4-methylphenyl, 2,6-dimethylphenyl, 2,6-diethylphenyl, 4-butylphenyl, 2-trifluoromethylphenyl, 2-ethoxyphenyl, 4-phenylphenyl, 4-phenoxyphenyl, N-methylbenzamidophenyl, N,N-diphenylcarbamoylphenyl, N,N-dibutylsulfamoylphenyl, N,N-diphenylsulfamoylphenyl, N-methylsulfonamidophenyl, 2-methyl-5-nitrophenyl, 2-chloro-5-cyanophenyl, 5-chloro-2-methylphenyl, 2,6-dichloro-4-methylphenyl, 2,4-dichloro-6-methylphenyl, 2-chloro-4,6-dimethylphenyl, 2,6-dichloro-4-methoxyphenyl, 2,6-dichloro-4-nitrophenyl, 2,4,6-trimethyl-3-nitrophenyl, 2,4,6-trimethyl-3-acetamidophenyl, 2,4,6-trimethyl-3-[ $\alpha$ -(2,4-di-*tert*-amylphenoxy)butylamido]phenyl and the like.

Among the 3-ureido-5-pyrazolones represented by general formula I, the couplers of the formula in which at least one orthoposition of the phenyl group represented by  $R_2$  has been substituted by a halogen atom, an alkyl group having 1-5 carbon atoms, or an alkoxy group having 1-5 carbon atoms is particularly preferred.

Specific examples of the group  $R_1$  of general formula I include alkyl groups such as methyl, ethyl, propyl, isopropyl, butyl, iso-butyl, tert-butyl, amyl, hexyl, octyl, decyl, dodecyl, pentadecyl, octadecyl, allyl, heptadec-

nyl, and benzyl groups, and aryl groups such as phenyl and tolyl groups.

The phenyl groups having the following substituents are used as the group R<sub>1</sub> of general formula I;



In the above formulae, R<sub>3</sub>, R<sub>5</sub>, R<sub>7</sub>, R<sub>8</sub>, R<sub>9</sub>, R<sub>11</sub> and R<sub>12</sub> each represents an alkyl group; R<sub>4</sub>, R<sub>6</sub> and R<sub>10</sub> each represents a hydrogen atom or an alkyl group; and n is an integer of 1-5. Generally, any alkyl group for the moieties R<sub>3</sub> to R<sub>12</sub> listed above will have from 1 to 18 carbon atoms, and for practical purposes are preferably unsubstituted.

It is preferred that at least one of R<sub>1</sub> and R<sub>2</sub> of general formula I have a ballast group making the coupler non-diffusible. As is known in the art, ballast groups are hydrophobic groups usually containing 8 to 32 carbon atoms.

Examples are described in U.S. Pat. Nos. 2,600,788; 2,865,751; 3,337,344 and 3,418,129, and Japanese Patent Publications 27563/64 and 19035/70.

Specific examples of the 3-ureido-5-pyrazolone couplers are illustrated below:

Coupler - 1



Coupler - 2



Coupler - 3



Coupler - 4



Coupler - 5



Coupler - 6



Coupler - 7



Coupler - 8



Coupler - 9



Coupler - 10



Coupler - 11



3,861,923

9

10

Coupler - 12



Coupler - 13



Coupler - 14



Coupler - 15



3,861,923

11

Coupler - 16



12



Coupler - 17



Coupler - 18



Coupler - 19



Coupler - 20



Coupler - 21



Coupler - 22



Coupler - 23



Coupler - 24



The 3-ureido-5-pyrazolone couplers used in this invention can be prepared according to the methods described in U.S. Pat. No. 3,558,319; and Japanese Patent Applications 100911/1970; 106716/1970, etc.

In the silver halide emulsion of this invention, the abovementioned 3-ureido-5-pyrazolone couplers can be used alone or as a combination of two or more cou-

plers. Furthermore, the 3-ureido-5-pyrazolone coupler may be used together with other two-equivalent or four-equivalent couplers. These couplers are sometimes called colorless couplers, colored couplers or DIR couplers, and specific examples of them include the couplers described in U.S. Pat. Nos. 2,455,170; 2,600,788; 2,908,573; 3,062,653; 3,148,062;

3,227,551; 3,227,554; 3,418,129; 3,516,831; 3,519,429; and 3,617,291.

The 3-ureido-5-pyrazolene couplers of the present invention, whether used singly or as a combination of two or more thereof, are not particularly limited in proportions so long as the objects of the present invention are met. However, generally speaking, they will be used in an amount of from about 20 to about 100 percent by weight, preferably 50 to 100 percent by weight, of the total amount of magenta color forming couplers used.

Those color couplers are introduced into a hydrophilic colloid as is typically used for photographic materials according to any known method. For instance, they can be dispersed in a hydrophilic colloid using a high boiling point organic solvent such as dibutyl phthalate and tricresyl phosphate as described in U.S. Pat. No. 2,322,027 and/or a low-boiling point organic solvent such as ethyl acetate and tetrahydrofuran as described in U.S. Pat. Nos. 2,801,170; 2,801,171; and 2,946,360.

The aldehydes used together with the 3-ureido-5-pyrazolone coupler according to the present invention include compounds having an alkyl group, an aryl group, or a heterocyclic group bonded to the aldehyde group, i.e., aliphatic aldehydes, aromatic aldehydes or heterocyclic aldehydes can be used in the present invention. The aliphatic aldehydes preferably contain from 2 to 20 carbon atoms, most preferably 2 to 8 carbon atoms. Among the aromatic aldehydes, most preferred are those containing a formyl group attached to the phenyl or naphthyl ring, though aryl substituted with halogen, nitro, hydroxy,  $C_1$ - $C_8$  alkyl,  $C_1$ - $C_8$  alkoxy, allyl, carboxy, sulfo and the like are also useful.

Among the aldehydes, benzaldehydes with or without the above substituents are preferred.

Specific examples of such compounds are acetaldehyde, propionaldehyde, butylaldehyde, isobutylaldehyde, pivalylaldehyde, heptaldehyde, laurin aldehyde, stearinaldehyde, succindialdehyde, crotonaldehyde, benzaldehyde, o-chlorobenzaldehyde, m-chlorobenzaldehyde, p-chlorobenzaldehyde, p-bromobenzaldehyde, p-nitrobenzaldehyde, p-hydroxybenzaldehyde, o-tolualdehyde, cinnamaldehyde,  $\alpha$ -naphthaldehyde and furfural, etc.

Those aldehydes can be used alone or as a combination of two or more of such aldehydes. The addition amount of the aldehyde is usually about 0.05 to about 30 mols, in particular about 0.1 mol to about 10 mols, per mol of the coupler.

It is preferred that the aldehyde be added to a hydrophilic colloid when preparing the coupler dispersion by adding the above-described coupler or couplers to the hydrophilic colloid together with the aforesaid high boiling point organic solvent and/or the low boiling point organic solvent. Alternatively, they can be added to a silver halide emulsion at the preparation of coating compositions together with the coupler dispersion, a hardening agent, a stabilizer, a wetting agent, etc.

The amount of magenta forming coupler in accordance with the present invention is not limited so long as, of course, the color photographic material of the present invention meets the objects heretofore recited, that is, yields a magenta dye image of good heat and moisture resistance. However, since commercially it is necessary to provide an element which will provide results pleasing to the vast majority of purchasers, generally the amount of magenta color forming coupler will

be from about 0.05 to about 0.5 moles per mole of silver halide, most preferably, 0.07 to 0.2 moles per mole of silver halide.

Any known hydrophilic colloid(s) as are used in the color photographic art can be used as the hydrophilic colloid for the silver halide photographic emulsion layer of this invention. Preferred examples of such hydrophilic colloids are gelatin, albumin, gum arabic, agar agar, cellulose derivatives (such as alkyl esters of 10 carboxymethyl cellulose, hydroxyethyl cellulose, carboxymethyl hydroxyethyl cellulose, etc.), and synthetic resins (such as polyvinyl alcohol, polyvinyl pyrrolidone, etc.). These hydrophilic colloids are also preferably used as the binders for layers of the photographic material other than the silver halide emulsion layers, such as a protective layer, a filter layer, an intermediate layer, an antihalation layer, a subbing layer, a backing layer, etc.

The hydrophilic colloids used in various layers of the photographic material of this invention can be effectively hardened by hardening agents such as 1,4-dioxanes, aziridines, iso-oxazoles, active halogens, active vinyl compounds, etc. Typical examples of such hardening agents are described in U.S. Pat. Nos. 3,232,764; 3,288,775; 2,732,303; 3,635,718; 3,232,763; 2,732,316; 2,586,168; 3,103,437; 3,017,280; 2,983,611; 2,725,294; 2,725,295; 3,100,704; 3,091,537; 3,321,313 and 3,543,292 and British Pat. Nos. 974,723; 1,167,207 and 994,869.

In the present invention any silver halide emulsion as is usually used in the field of photography, such as a silver bromide emulsion, silver iodobromide emulsion, silver chloroiodobromide emulsion, silver chlorobromide emulsion and silver chloride emulsion can be used. Also, the so-called converted halide type silver halide emulsions as described in, e.g., U.S. Pat. No. 3,622,318 and British Pat. No. 635,841, can be used.

A preferred average gain size for the silver halide is from about 0.05 to about 1.5 microns. The weight ratio 40 of silver halide to binder most suitably ranges from about 0.2 to about 20 (silver halide/binder), preferably about 0.3 to about 5 in the layer. These values are not limitative, but provide a most superior element.

The silver halide emulsions (used in the color photographic materials) of this invention can be chemically sensitized by active gelatin or a sulfur compound according to the process described in U.S. Pat. Nos. 1,574,944; 1,623,499 and 2,410,869. They can also be sensitized by a noble metal salt such as a palladium or a gold salt as described in U.S. Pat. Nos. 2,448,060; 2,399,083 and 2,642,361. Furthermore, they can be sensitized by a reducing agent such as a stannous salt as described in U.S. Pat. No. 2,487,850, or sensitized by a polyalkylene derivative. They can also be spectrally sensitized by a cyanine by or merocyanine dye such as described in U.S. Pat. Nos. 2,519,001; 2,666,761; 2,734,900; 2,739,964 and 3,481,742.

The silver halide emulsion of this invention can contain a stabilizer such as a mercury compound, mercaptotetrazole, thiazole, azaindene, etc.; a plasticizer such as glycerin, latex, etc.; and a wetting agent such as saponin, polyethylene glycol monolauryl ether, etc. Furthermore, the silver halide emulsion can contain an antistatic agent, an ultraviolet absorbent, a fluorescent whitening agent, dyes, etc.

The silver halide emulsion containing the 3-ureido-5-pyrazolone and the aldehyde compound according to

this invention is effectively used as a green-sensitive emulsion layer in an ordinary multi-layer color photographic material. In this case, the order of the photosensitive emulsion layers may be, from the support side, a red-sensitive emulsion layer, a green-sensitive emulsion layer and a blue-sensitive emulsion layer, or may be a blue-sensitive emulsion layer, red-sensitive emulsion layer and a green-sensitive emulsion layer.

In addition to these photosensitive emulsion layers, the color photographic material of this invention can have an antihalation layer, intermediate layer(s), filter layer, protective layer, etc.

The support for the photographic materials of this invention on which the photosensitive silver halide emulsion layers are formed is preferably a cellulose ester film such as a cellulose nitrate film, a cellulose acetate film, etc.; a polyester film such as a polyethylene terephthalate film; a polyvinyl chloride film; a polystyrene film; a polycarbonate film; a baryta-coated paper; a resin-coated paper, and the like. This listing is, of course, not limitative.

The color photographic material of this invention is imagewise exposed in an ordinary way and then processed according to usual color photographic proceedings. The main processing steps are a color development, a bleach and a fix and, if necessary, a washing step may be applied between each step. After fixing, the color photographic material is washed and dried but it is desirable to process the color photographic material in a stabilization bath prior to drying.

As is known to those skilled in the art, photographic processing temperatures typically range from about 20°C or less to 60°C or higher. Temperatures of about 30°C or higher are suitable for high speed processing procedures. Processing times for each processing step can vary widely, depending on the processing temperature, but usually range from several seconds to several minutes or more.

Useful color developers are aqueous alkaline solutions containing a color developing agent. As the color developing agent, all known primary aromatic amine dye-forming developing agents can be used. Examples of such color developing agents are phenylenediamines such as N,N-diethyl p-phenylenediamine, N-ethylhydroxyethyl p-phenylenediamine, N-ethyl-N-hydroxyethyl-2-methyl p-phenylenediamine, N-ethyl-β-N-methane sulfoneamidoethyl-3-methyl-4-aminoaniline, N,N-diethyl-2-methyl-p-phenylenediamine, and sulfates, hydrochlorides, sulfides, etc., thereof. See C. E. K. Mees and T. H. James, *The Theory of the Photographic Process*, pages 294-295 (The Macmillan Co., 1966), and U.S. Pat. Nos. 2,592,364 and 2,193,015. The color developer used for developing the color photographic material of this invention may further contain ordinary additives as are used in this art such as a sulfite of an alkali metal, a carbonate, a bisulfite, a bromide, an iodide, benzyl alcohol, etc.

The bleach solution can contain any known bleaching agent such as ferricyanide, bichromate, etc. Also, the fix solution can contain any known fixing agent such as sodium thiosulfate, potassium thiocyanate, etc. Furthermore, the bleach step and the fix step can be conducted in one bath, and such a "blix" bath is described in, e.g., U.S. Pat. No. 3,582,322.

Typical bleach agents are discussed in detail in the *Journal of the Society of Motion Picture and Television*

Engineers 61, 667-701 and U.S. Pat. No. 3,189,452; typical fix agents in Mason, *Photographic Processing Chemistry*, pages 187-188, Focal Press (1966); and typical blix solutions in German Pat. Nos. 866,605 and 966,410, in *British Journal of Photography*, pages 122-123 and 126 (1966) and in U.S. Pat. No. 3,582,322. These references also disclose generally used proportions.

The photographic material of this invention provides stable color images which are not faded if the photographic material is exposed to heat or moisture or stored for a long period of time. This merit is obtained by the combination of the 3-ureido-5-pyrazolone and the aldehyde as mentioned above without using formalin, i.e., since the aldehydes of the present invention are limited to those having an aldehyde group bonded to a carbon atom, formaldehyde is excluded from the scope of the present invention. This is quite astonishing upon considering that if the aforesaid aldehyde is used together with 3-acylamino-5-pyrazolone, the stability of the color images cannot be improved.

Furthermore, the aldehyde used in this invention does not have a harmful influence on the photographic properties, e.g., hindering the coupling of couplers and causing stain as in the case of using formalin or a compound releasing formalin.

Moreover, the aldehyde in this invention has the effect of preventing the formation of magenta development fog. Further, changes in sensitivity of the photosensitive emulsion of this invention during storage is prevented. This effect is further observed in the emulsion layers formed over or under the silver halide emulsion layer of this invention, and is a surprisingly effect.

The invention will now be explained in further detail by the following examples.

#### EXAMPLE 1

To 100 g of a gelatino silver chlorobromide emulsion containing 50 mol percent of bromide and 0.05 mol of silver, there were added a sensitizing dye having its sensitization maximum at about 545 m $\mu$  (150 mg per mole of silver halide) and 60 g of a coupler dispersion prepared by dispersing the following compositions by means of a homogenizer. The resulting silver halide emulsion was coated on a baryta-coated paper (coated amount of silver  $6 \times 10^{-3}$  mol/m $^2$ ). Thus, samples A-D were prepared.

|    | Coupler dispersion                                     | A      | B      | C      | D      |
|----|--------------------------------------------------------|--------|--------|--------|--------|
| 40 | Coupler 1 (earlier set out)                            | 100 g  | 100 g  | 100 g  | —      |
| 45 | Coupler A (known)                                      | —      | —      | —      | 100 g  |
| 50 | Dibutyl phthalate                                      | 100 g  | 100 g  | 100 g  | 100 g  |
| 55 | Ethyl acetate                                          | 200 g  | 200 g  | 200 g  | 200 g  |
| 60 | 10% aqueous gelatin solution                           | 1000 g | 1000 g | 1000 g | 1000 g |
| 65 | Aqueous solution of 5% sodium dodecylbenzene sulfonate | 50 g   | 50 g   | 50 g   | 50 g   |
|    | Acetaldehyde                                           | —      | 6 g    | —      | —      |
|    | Heptaldehyde                                           | —      | —      | 5 g    | —      |

Known coupler A: the condensation product of 1-phenyl-3-[3-(2-carboxymethylicos-3-enamide)-benzamido]-5-pyrazolone and acetaldehyde described in U.S. Pat. No. 3,468,666.

Each of the samples thus prepared was stagewise exposed (1,000 lux, 1 sec.) through a green filter trans-

mitting light of 500-600 m $\mu$  and a silver wedge and then processed as follows:

| Processing step   | temperature | time   | 5 | Sample | Maximum density     | Dye remaining percentage |
|-------------------|-------------|--------|---|--------|---------------------|--------------------------|
|                   |             |        |   |        | initial density 0.5 | initial density 1.5      |
| Color development | 30°C        | 4 min. |   | A      | 2.5                 | 45                       |
| Blix              | 30°C        | 2 min. |   | B      | 2.5                 | 85                       |
| Washing           | 30°C        | 2 min. |   | C      | 2.5                 | 87                       |
| Stabilization     | 30°C        | 2 min. |   | D      | 1.7                 | 55                       |

The compositions of the processing solutions used in the processings were as shown below:

|                                                                    |          |  |  |  |
|--------------------------------------------------------------------|----------|--|--|--|
| Color developer                                                    |          |  |  |  |
| sodium metaborate                                                  | 25 g     |  |  |  |
| sodium sulfite                                                     | 2 g      |  |  |  |
| hydroxylamine (sulfate)                                            | 2 g      |  |  |  |
| potassium bromide                                                  | 0.5 g    |  |  |  |
| 6-nitrobenzimidazole (nitrate)                                     | 0.02 g   |  |  |  |
| sodium hydroxide                                                   | 4 g      |  |  |  |
| benzyl alcohol                                                     | 15.8 ml  |  |  |  |
| diethylene glycol                                                  | 20 ml    |  |  |  |
| N-ethyl-N- $\beta$ -(methanesulfone-amidoethyl)-p-phenylenediamine | 8 g      |  |  |  |
| water to make                                                      | 1000 ml. |  |  |  |
| Blix solution:                                                     |          |  |  |  |
| iron salt of ethylenediamine-tetraacetic acid                      | 45 g     |  |  |  |
| ammonium thiocyanate                                               | 10 g     |  |  |  |
| sodium sulfite                                                     | 10 g     |  |  |  |
| ammonium thiosulfate (60%)                                         | 100 ml   |  |  |  |
| tetrasodium ethylenediamine-tetraacetate                           | 5 g      |  |  |  |
| water to make                                                      | 1000 ml. |  |  |  |
| Stabilizing bath:                                                  |          |  |  |  |
| tartaric acid                                                      | 10 g     |  |  |  |
| zinc sulfate                                                       | 10 g     |  |  |  |
| sodium metaborate                                                  | 20 g     |  |  |  |
| water to make                                                      | 1000 ml. |  |  |  |

After measuring the reflection density of the magenta dye images thus formed, the processed samples were stored for 14 days at 60°C and 70 percent relative humidity to conduct a fading test and then the reflection density of the dye images was again measured. The percentage of dye remaining in the portions having image densities of 0.5 and 1.5 before the fading test were calculated by the following equation and are shown in Table 1.

$$\text{Dye remaining percentage} = (A/B) \times 100$$

A: dye density after fading test - fog density after fading test.

B: dye density before fading test - fog density before fading test.

20  
TABLE 1

|    |        |                     |                          |
|----|--------|---------------------|--------------------------|
| 10 | Sample | Maximum density     | Dye remaining percentage |
|    |        | initial density 0.5 | initial density 1.5      |
|    | A      | 2.5                 | 60                       |
|    | B      | 2.5                 | 90                       |
|    | C      | 2.5                 | 90                       |
|    | D      | 1.7                 | 65                       |

15 Sample B and C containing the 3-ureido-5-pyrazolone coupler and the aldehyde according to this invention gave stable magenta dye images which caused less fading, and this tendency was particularly remarkable at the low density portions. On the other hand, Sample D containing the known coupler gave insufficient coupling density and gave unstable dye images.

20  
EXAMPLE 2

A subbing layer was formed on a cellulose acetate film support having an antihalation layer containing carbon black on the opposite side, and then a coating composition containing a silver iodobromide emulsion containing 1.2 mol percent iodine and a coupler dispersion prepared by dispersing a yellow coupler,  $\alpha$ -(2-methylbenzoyl)-3-[ $\alpha$ -(2,4-di-tert-amylphenoxy)acetamido]acetanilide using dibutyl phthalate and ethyl acetate was coated on the subbing layer to form a blue-sensitive layer. A gelatin intermediate layer was formed on the blue-sensitive layer and a coating composition containing a gelatino silver chlorobromide emulsion containing 30 mol percent bromide and spectrally sensitized so that it had its sensitization maximum at about 685 m $\mu$ , and a coupler dispersion prepared by dispersing a cyan coupler, 1-hydroxy-4-chloro-N-hexadecyl-N-(2-cyanoethyl)-2-naphthamide using butyl phthalate and ethyl acetate was coated on the intermediate layer to form a red-sensitive layer. A gelatin intermediate layer was coated on the red-sensitive layer and then a coating composition containing 100 g of silver chlorobromide (containing 0.06 mol of silver) containing 35 mol percent bromide and spectrally sensitized so that it had its sensitization maximum at about 555 m $\mu$ , and 250 g of a coupler dispersion prepared by dispersing the following components by means of a homogenizer was coated on the intermediate layer to 40 form a green-sensitive layer. A gelatin protective layer was coated on the emulsion layer. Samples E-I were thus prepared. All systems were gelatino systems.

| Coupler dispersion                                  | E      | F      | G      | H      | I      |
|-----------------------------------------------------|--------|--------|--------|--------|--------|
| Coupler 10 (earlier described)                      | 50 g   | 50 g   | 50 g   | 50 g   | —      |
| Known coupler B                                     | 50 g   | 50 g   | 50 g   | 50 g   | 100 g  |
| Dibutyl phthalate                                   | 50 g   | 50 g   | 50 g   | 50 g   | 50 g   |
| Ethyl acetate                                       | 200 g  | 200 g  | 200 g  | 200 g  | 200 g  |
| 10% aq. gelatin solution                            | 1000 g | 1000 g | 1000 g | 1000 g | 1000 g |
| aq. solution of 5% sodium dodecyl-benzene sulfonate | 100 g  | 100 g  | 100 g  | 100 g  | 100 g  |
| Benzaldehyde                                        | —      | 3 g    | —      | —      | —      |
| p-Chlorobenzaldehyde                                | —      | —      | 4 g    | —      | 4 g    |
| p-Nitrobenzaldehyde                                 | —      | —      | —      | 4 g    | —      |

Known coupler B: 1-(2,4,6-trichlorophenyl)-3-3-[ $\alpha$ -(2,4-di-tert-amylphenoxy)butylamido]benzamido-5-pyrazolone.

Each of the samples was exposed as in Example 1 and subjected to the following processings:

| Processing step     | temperature | time           |
|---------------------|-------------|----------------|
| Pre-processing bath | 27°C        | 10 sec.        |
| Washing             | do.         | 15 sec.        |
| Color development   | do.         | 5 min. 20 sec. |
| Washing             | do.         | 15 sec.        |
| Blix                | do.         | 4 min.         |
| Washing             | do.         | 2 min.         |
| Stabilization       | do.         | 10 sec.        |

The compositions of the processing solutions used in the steps were as follows:

|                                                   |          |  |
|---------------------------------------------------|----------|--|
| Pre-processing bath:                              |          |  |
| water                                             | 800 ml   |  |
| sodium carbonate (monohydrate)                    | 10 g     |  |
| sodium sulfate (anhydrous)                        | 50 g     |  |
| water to make                                     | 1000 ml. |  |
| Color developer:                                  |          |  |
| water                                             | 800 ml   |  |
| sodium hexametaphosphate                          | 2 g      |  |
| anhydrous sodium sulfite                          | 4 g      |  |
| 2-amino-5-diethylaminotoluene                     |          |  |
| hydrochloride                                     | 3 g      |  |
| sodium carbonate (monohydrate)                    | 2.5 g    |  |
| potassium bromide                                 | 2.0 g    |  |
| water to make                                     | 1000 ml. |  |
| Blix solution:                                    |          |  |
| sodium iron(III) ethylene-diaminetetraacetic acid | 34 g     |  |
| sodium carbonate (monohydrate)                    | 11 g     |  |
| borax                                             | 45 g     |  |
| sodium thiosulfate                                | 140 g    |  |
| water to make                                     | 1000 ml. |  |
| Stabilization bath:                               |          |  |
| water                                             | 800 ml   |  |
| polyethylene glycol (MW.400)                      | 5 ml     |  |
| 40% aqueous solution                              |          |  |
| water to make                                     | 1000 ml. |  |

After measuring the transmission density of the magenta dye images thus formed, the processed samples were stored for 30 days at 50°C and 70% relative humidity and then the transmission density of the dye images was again measured. The dye remaining percentages of the portions having image densities of 0.5 and 2.0 before the fading test are shown in Table 2, with all values being calculated as in Example 1.

TABLE 2

| Sample | Fog density | Dye remaining percentage |                     |
|--------|-------------|--------------------------|---------------------|
|        |             | initial density 0.5      | initial density 2.0 |
| E      | 0.08        | 50                       | 70                  |
| F      | 0.07        | 85                       | 90                  |
| G      | 0.06        | 87                       | 91                  |
| H      | 0.06        | 88                       | 93                  |
| I      | 0.08        | 58                       | 70                  |

From the above results, it will be understood that in samples F, G, and H of this invention, stable magenta dyes causing less fading of dye images were obtained, and further the occurrence of magenta development fog was suppressed. On the other hand, in the comparison sample I in which the 3-acylamino-5-pyrazolone magenta coupler and the aldehyde of this invention were used, the fading of the dye image was great. That is to

say, it will be understood that the use of the aldehyde in this invention was only effective in the combination with the 3-ureido-5-pyrazolone.

## EXAMPLE 3

On the surface of a paper, both surfaces of which were laminated with polyethylene containing titanium dioxide, a coating composition containing a silver chlorobromide containing 85 mol percent of bromine and a coupler dispersion prepared by dispersing a yellow coupler,  $\alpha$ -(4-methoxybenzyl)-3-[ $\alpha$ -(2,4-di-tert-amylphenoxybutylamide)]-6-chloroacetoanilide, using dibutyl phthalate and ethyl acetate, was coated to form a blue-sensitive layer. A gelatin intermediate layer was formed on the blue-sensitive layer. On the intermediate layer, a coating composition containing 100 g of silver chlorobromide emulsion (containing 0.07 mol of silver) containing 30 mol percent bromine and 100 g of a coupler dispersion prepared by dispersing a sensitizing dye having its sensitization maximum at about 545 m $\mu$  and the components shown below by means of a homogenizer was coated in a coated silver amount of  $1 \times 10^{-2}$  mol/m $^2$ .

| Coupler dispersion           | J      | K      | L      | M      |
|------------------------------|--------|--------|--------|--------|
| Coupler 10                   | 50 g   | 50 g   | 50 g   | 50 g   |
| Coupler 11                   | 50 g   | 50 g   | 50 g   | 50 g   |
| Dibutyl phthalate            | 100 g  | 100 g  | 100 g  | 100 g  |
| Ethyl acetate                | 150 g  | 150 g  | 150 g  | 150 g  |
| 10% Aqueous gelatin solution | 1000 g | 1000 g | 1000 g | 1000 g |
| Isopropylaldehyde            | —      | 5 g    | —      | —      |
| m-Chlorobenzaldehyde         | —      | —      | 5 g    | —      |
| p-Nitrobenzaldehyde          | —      | —      | —      | 5 g    |

A gelatin intermediate layer containing an ultraviolet absorbent, 2-(2'-hydroxy-3'-methyl-5'-sec-butylphenyl)benzotriazole, was coated on the emulsion layer and further, on the intermediate layer, a coating composition containing silver chlorobromide containing 40 mol percent bromine and a coupler dispersion prepared by dispersing a cyan coupler, 4,6-dichloro-3-methyl-2-[ $\alpha$ -(2,4-di-tert-amylphenoxy)acetamido]phenol, using dibutyl phthalate and ethyl acetate, was coated. Finally, a gelatin protective layer was coated on the emulsion layer. Samples J-M were thus prepared.

Directly after the preparation of the samples and after storing the samples for 3 days at 40°C and 80% relative humidity, the samples were wedge exposed using a filter transmitting light of 500-600 m $\mu$  and a filter transmitting light have wave lengths longer than 600 m $\mu$ , and then processed as in Example 1. The red sensitivity and the green sensitivity of the various samples thus processed were measured, and from the results the change in sensitivity with the storage under high-temperature and high-humidity conditions was determined. The results are shown in Table 3, in which the value “-0.30” shows that the sensitivity of the sample measured was reduced by 0.30 (in logarithmic units) as compared with the sensitivity of the fresh sample. Also, the fog density and the results of a fading test conducted as in Example 1 are shown in the same table.

TABLE 3

| Sample | Change of sensitivity |             | Fog density | Dye remaining percent |                     |
|--------|-----------------------|-------------|-------------|-----------------------|---------------------|
|        | Red sens.             | Green sens. |             | Initial density 0.5   | initial density 1.0 |
| J      | -0.30                 | -0.70       | 0.13        | 45                    | 60                  |
| K      | -0.15                 | -0.50       | 0.12        | 80                    | 85                  |
| L      | -0.15                 | -0.50       | 0.12        | 85                    | 90                  |
| M      | -0.15                 | -0.50       | 0.11        | 90                    | 95                  |

From the above results, it will be understood that the stability of the magenta images was improved by this invention, and further the fog density of the magenta layer was lowered and the change of the sensitivity of the green-sensitive layer itself, as well as the sensitivity of the red-sensitive layer were minimized by this invention when the samples of this invention were stored under high temperature and high-humidity conditions.

Thus, the excellent points of the color photographic materials of this invention will be understood from the above examples.

While the invention has been described in detail and with reference to specific embodiments thereof, it will be apparent to one skilled in the art that various changes and modifications can be made therein without departing from the spirit and scope thereof.

What we claim is:

1. A color photographic material which provides magenta dye images of excellent heat and moisture resistance and reduced magenta development for comprising a support having thereon a silver halide photographic emulsion layer containing a 3-ureido-5-pyrazolone magenta coupler and a compound having an aldehyde group bonded to a carbon atom; 35

wherein said magenta coupler is a compound represented by the formula



wherein R<sub>1</sub> represents an alkyl group or an aryl group and R<sub>2</sub> represents a phenyl group; and

wherein said aldehyde group is bonded to the carbon atom of an alkyl group, an aryl group or a furfural group, wherein said alkyl group contains from 2-20 carbon atoms and said aromatic group is a formyl-substituted phenyl or naphthyl ring.

2. A color photographic material as set forth in claim 1 wherein  $R_1$  is a  $C_1$ – $C_{32}$  carbon atom alkyl group or a monoaryl group and  $R_2$  is a phenyl group.

3. A color photographic material as set forth in claim 2 wherein  $R_1$  is a  $C_8$ – $C_{18}$  carbon atom alkyl group, a phenyl group or a tolyl group.

4. A color photographic material as set forth in claim 1 wherein  $R_2$  is a phenyl group substituted with a halogen atom, a  $C_1-C_5$  alkyl group or a  $C_1-C_5$  alkoxy group.

5. The color photographic material as set forth in claim 1 wherein at least one of  $R_1$  and  $R_2$  has a ballast group.

6. A color photographic material as set forth in claim 5 wherein the ballast group is a  $C_8$ - $C_{32}$  hydrophobic group.

7. A color photographic material as set forth in claim 1 wherein the amount of magenta dye-forming coupler is from about 0.05 to about 0.5 moles per mole of silver halide in the emulsion.

8. A color photographic material as set forth in claim 7 wherein the amount of magenta dye-forming coupler is from about 0.07 to about 0.2 moles per mole of silver halide in the emulsion.

9. The color photographic material as set forth in claim 7 wherein the proportion of said compound having an aldehyde group bonded to a carbon atom is from 0.05 mol to about 30 mols per mol of said magenta coupler.

10. A color photographic material as set forth in claim 1 wherein the alkyl group bonded to a carbon atom contains from 2 to 20 carbon atoms, and the aromatic group bonded to a carbon atom is a formyl-substituted phenyl or naphthyl ring.

11. A color photographic material as set forth in claim 1, wherein said aryl group bonded to said aldehyde group is substituted with halogen, nitro, hydroxy,  $C_1$  -  $C_8$  alkyl,  $C_1$  -  $C_8$  alkoxy, aryl, carboxy or sulfo.

12. A color photographic material as set forth in claim 1 wherein the aldehyde is a benzaldehyde.

13. A color photographic material as set forth in claim 12 wherein the benzaldehyde is substituted with halogen, nitro, hydroxy,  $C_1$  -  $C_8$  alkyl,  $C_1$  -  $C_8$  alkoxy, aryl, carboxy or sulfo.

14. A color photographic material as set forth in claim 1 where the compound having an aldehyde group is selected from the group consisting of acetaldehyde, propionaldehyde, butylaldehyde, iso-butylaldehyde, pivalylaldehyde, heptaldehyde, laurinaldehyde, stearinaldehyde, succindialdehyde, crotonaldehyde, benzaldehyde, o-chlorobenzaldehyde, m-chlorobenzaldehyde, p-chlorobenzaldehyde, p-bromobenzaldehyde, p-nitrobenzaldehyde, p-hydroxybenzaldehyde, o-tolualdehyde, cinnamaldehyde,  $\alpha$ -naphthaldehyde or furfural.

15. A color photographic material as set forth in claim 14 wherein the average grain size of the silver halide present in the emulsion is from about 0.05 to about 1.5 microns.

16. A color photographic material as set forth in claim 15 wherein the weight ratio of silver halide to binder is from about 0.2 to about 20 (silver halide-binder).

17. A color photographic material as set forth in claim 1 wherein  $R_1$  is an alkyl group.

18. A color photographic material as set forth in claim 1 wherein  $R_1$  is an aryl group.

19. A color photographic material as set forth in claim 1 wherein  $R_1$  is a phenyl group selected from:

(a)  $-\text{NHCO}R_3$

(b)  $-\text{NHCO}\left\{ \text{CH}-\text{O}-\text{C}_6\text{H}_4-\text{R}_5 \right\}_n-\text{R}_6$

(c)  $-\text{NHCOCH}_2\text{CH}_2-\text{N}(\text{COR}_7)-\text{R}_8$

**25**

, wherein  $\text{R}_3$ ,  $\text{R}_5$ ,  $\text{R}_7$ ,  $\text{R}_8$ ,  $\text{R}_9$ ,  $\text{R}_{11}$ , and  $\text{R}_{12}$  each represent an alkyl group, and  $n$  is an integer of 1-5.

10

**26**

20. A color photographic material as set forth in claim 19 wherein any of  $\text{R}_3$ - $\text{R}_{12}$  has from 1 to 18 carbon atoms.

21. A color photographic material as set forth in claim 1 wherein said silver halide photographic emulsion is a silver halide gelatino photographic emulsion, further containing said magenta coupler and said compound having an aldehyde group.

\* \* \* \* \*

15

20

25

30

35

40

45

50

55

60

65